

## UNITED STATES PATENT OFFICE

2,564,022

## MANUFACTURE OF SYNTANS FROM VANILLIN AND LEATHER TANNED THEREWITH

John Miglarese, Cincinnati, Ohio, assignor to The United States Leather Company, New York, N. Y., a corporation of New Jersey

No Drawing. Application September 8, 1948,  
Serial No. 48,322

2 Claims. (Cl. 260—49)

1

My invention relates to a novel type of syntan made from vanillin and to the surprising results of the use of such syntan.

In the preparation of syntans it has been proposed to make a syntan by treating the concentrated sulphonation mixture (including unchanged sulphuric acid) of phenol sulphonic acid with formaldehyde at a temperature of 30 to 35° C. (Bureau of Standards Technological Papers, vol. 20, No. 309, by Edward Wolensensky). Thus 10 the use of phenol sulfonated aldehyde compounds as syntans is broadly old and well known.

So far as I am advised, however, the use of benzaldehydes in a relatively pure state condensed with phenol and sulfuric acid has not been proposed.

It is my object to prepare a syntan from a relatively non-complex benzaldehyde material such as vanillin. The chemical formula of vanillin is  $(\text{OH})(\text{CH}_3\text{O})\text{C}_6\text{H}_3\text{CHO}$ , 4 hydroxy 3 methoxy benzaldehyde and it has the structural formula



Vanillin may be produced as a degradation product of lignin.

An object of my invention is to utilize vanillin because its unique composition consisting of a phenolic group and an aldehyde group which are available to make a syntan, rich in phenolic groups, contribute surprisingly good leathering characteristics in tanning.

Another object of my invention is to make a leathering material practically in one step without the use of expensive equipment, merely by dissolving the phenol and vanillin and sulfonating, causing simultaneous sulfonation and condensation of the phenolic aldehyde and phenol, to a tanning material as follows:

*Example 1*

One mol of vanillin and two mols of phenol are dissolved in each other, and 1½ mols of sulfuric acid (98%) is added with stirring in the course of 1½ hour. Permit the temperature to rise of its own exothermic reaction. Stir for 1½ hours, add ½ its weight of 5% lactic acid and neutralize the mass to a pH of 3.5 with sodium hydroxide which is ready for use in tanning.

2

*Example 2*

Condense 75.2 grams of phenol with 60.8 grams of vanillin (about 2 mols of phenol to 1 of vanillin) and 5 grams of oxalic acid for 3 hours, at the end of which produces a resinous mass having a red color. 45–60 cc. of concentrated 98%  $\text{H}_2\text{SO}_4$  is added to the mass gradually. The mass is made less viscous by a water bath to facilitate stirring. The  $\text{H}_2\text{SO}_4$  is added in a period of ½ hour. The temperature is kept around 80°–90° and the mixture is stirred for one hour at this temperature. The red mass is diluted with its weight of water. 20 grams of concentrated hydroxy acetic acid is added to the mass. The whole is made of pH of 3.5 with caustic soda or sodium carbonate. The synthetic tanning extract is now ready to be used for tanning. A piece of depickled skin is introduced into the liquor having 3% tanning content and the ratio of the liquor to the hide or skin is 5 to 1. The skin or hide is permitted to stand in liquor until the tanning material has struck through. The leather is oiled, dried and finished having full 25 and excellent feel.

*Example 3*

The phenolic aldehyde, vanillin, can be used to condense 1 mol of phenol and 1 mol meta cresol 30 in the presence of sulfuric acid performed the same way as in Example 1. The presence of cresol gives a brownish red colored tanning product and a brown leather. The skin is tanned as in Example 2.

35 Comparative tests on the skin tanned in accordance with Example No. 2 with skins tanned with other types of syntans and with vegetable tanning reagents indicate a quality of tanning heretofore unknown. There is a fullness and plumpness and soft feel which makes the skin tanned in accordance with my invention as set forth herein, stand out as different in physical properties than leathers tanned in other ways.

40 45 Having thus described my invention, what I claim as new and desire to secure by Letters Patent is:

1. The method of producing a tanning material which comprises subjecting a mixture of a phenol and vanillin, in the proportions of about 50 2 mols of phenol to 1 of vanillin, to condensation and to sulfonation with concentrated sulfuric acid to form a water soluble condensation and sulfonated product and reducing the acidity 55 of the resulting product to a pH of around 3.5,

2. A synthetic tanning material produced in accordance with the process of claim 1.  
 JOHN MIGLARESE.

## REFERENCES CITED

The following references are of record in the file of this patent:

## UNITED STATES PATENTS

|           |        |                |    |           |
|-----------|--------|----------------|----|-----------|
| Number    | Name   | Date           | 10 | 2,191,737 |
| 1,430,477 | Tullis | Sept. 26, 1922 |    |           |

|   | Name     | Date          |
|---|----------|---------------|
|   | Schmidt  | May 26, 1925  |
|   | McIntosh | July 31, 1928 |
|   | Orthner  | May 12, 1936  |
| 5 | Alles    | Nov. 23, 1937 |
|   | Alles    | June 28, 1938 |
|   | Bauer    | Feb. 28, 1939 |
|   | Mauthe   | Dec. 26, 1939 |
|   | Wallace  | Jan. 29, 1940 |
|   | Alles    | Feb. 27, 1940 |